

1,626,230

April 26, 1927.

L. T. FREDERICK

COMPOSITE GEAR AND METHOD OF MAKING SAME

Filed Aug. 13, 1923



Inventor:  
Louis T. Frederick

By Cheever & Cox  
Attn: [unclear]

Patented Apr. 26, 1927.

1,626,230

# UNITED STATES PATENT OFFICE.

LOUIS T. FREDERICK, OF VALPARAISO, INDIANA, ASSIGNOR TO FIBROC INSULATION COMPANY, OF VALPARAISO, INDIANA, A CORPORATION OF INDIANA.

## COMPOSITE GEAR AND METHOD OF MAKING SAME.

Application filed August 13, 1923. Serial No. 657,181.

My invention relates to composite gears and methods of making the same. Gears of this nature are frequently referred to as "fiber" gears and consist of fibrous material and a binding substance such as a phenol condensation product of the general character set forth in Baekeland Patent 1,160,364. Laminated gears consisting of a woven fabric consolidated and held in compressed state by means of a phenol condensation product are not broadly new, being shown, for example, in Conrad Patent 1,167,743; but in that patent the gear wheel is of uniform thickness from center to circumference. It is desirable in many cases—especially in gears of the larger sizes or in gears of either large or small sizes in which the available room on the shaft is limited, and also in those cases where it is desired to lighten the gear—to reduce the thickness of the central portion of the gear, thus producing a rim section of the full width or thickness of the gear and a central or web section which is thinner. Various methods have been attempted for producing such gears having a reduced web section. According to one method the surplus material is machined away, but this method is expensive by reason of the waste of the material which is removed. According to another method, rings of fabric have been employed and these have been inter-leaved or alternated with the peripheral portion of complete discs, the rings thickening the rim portion and building up the gears at this part. This method, however, is defective in that the sheets of fabric are distorted during manufacture, and it is impossible, commercially speaking at least, to produce a gear wheel in which the cross section will be uniform. If it is not uniform the gear when rotating will tend to run out of true. The gear being unbalanced will have a tendency to "wobble" and this will result in excessive wear at certain points, thus rendering the gear noisy and short-lived. The object of my invention is to produce a gear having a web section of reduced thickness but which will lend itself to ready manufacture and will make it possible under commercial conditions to produce a gear in which the cross section on any given plane will be symmetrical and the sections on all diametral planes will be the same.

In carrying out my process I produce the

web section from a set of sheets of layers all lying in parallel planes and produce the thickened rim section by adding, outside of the web section, a plurality of rings arranged in parallel planes and held under compression by suitable binding means, preferably a phenol condensation product. According to one development of my method the web section layers and the ring layers are placed in a mold provided with means for producing differential pressures so that the rim section will receive an aggregate compression greater than the web section which contains fewer layers.

I accomplish my object in the manner illustrated in the accompanying drawings, in which—

Figure 1 is a view of a suitable type of mold shown in diametral section. In this figure the plungers or dies are shown in initial position, that is, at the beginning of their compressive action.

Figure 2 is similar to Figure 1 but shows the mold "closed up"—that is, with the dies in final position.

Figure 3 is a diametral section of a gear blank produced according to my process.

Figure 4 is a view partly in diametral section of a gear produced according to the process.

Figure 5 is a side view of the gear.

Figure 6 is a fragmentary view illustrating more or less diagrammatically the arrangement of the component parts of the gear.

Like numerals denote like parts throughout the several views.

I will describe the method in connection with a mold and press especially adapted for it. This consists of an outer cylindrical shell 1 having a lower ring plunger 2 and an upper ring plunger or die 3. Fitting within these plungers are cylindrical plungers 4 and 5. Plungers 4 and 5 are chambered to receive helical compression springs 6. The parts 1 and 2 normally rest upon any suitable platen or platform 7, and the pressure is obtained from the platen 10 of any suitable type of press. When operating upon phenol condensation products or binders of similar characters it is desirable to heat the platen in any appropriate manner, for example by steam pipes 12.

In carrying the mold I first place in it a plurality of rings 14 of fibrous material, for

example, cotton duck, the same being saturated in a binder, preferably a phenol condensation product, which will harden under heat. I next place in the mold a plurality 5 of discs 16 of the same material and then a plurality of rings 18 similar to the rings 14. At this time the shell 1, ring die 2 and lower spring 6 will rest upon the supporting platform. The parts are so proportioned 10 that the upper surface of die 4 will be above the level of the upper surface of ring 2. I then lower the upper ring 3 into position in the shell 1 and then lower the plunger 5 into position. The upper compression spring 6 15 is put in place, whereupon the mold is charged ready for the descent of the platen 10 of the press. The parts will then present the appearance shown in Figure 1, the ring 3 projecting above the upper surface of the 20 upper plunger 5, and the upper spring 6 contacting the lower surface of the platen. The mold is now ready to be closed up in the sense of being subjected to pressure.

As the platen 10 descends it exerts pressure upon all surfaces of the contents of the 25 mold. The pressure upon the rim portions formed by the rings 14 and 18 and intervening portion of the discs 16 is a direct unyielding pressure while the pressure of the 30 plungers 4, 5 upon the web section is a yielding pressure, as the springs 6 intervene between the stationary support and the platen 10. As the platen descends the springs yield and finally permit the lower plunger 4 to 35 reach the lower support and the platen 10 to reach the upper plunger 5. The platen continues to descend until the mold is entirely closed and the parts occupy the positions shown in Figure 2. A convenient method 40 for limiting the descent of the plunger is to so proportion the height of the shell 1 that the correct pressure will be attained when the platen seats upon the top of the shell as shown in Figure 2.

45 The parts are permitted to remain in this condition under heat until the fabric and its binder have been firmly consolidated, compressed and hardened, after which the plungers and the gear blank will be removed 50 and the press thus prepared for another charge. When the compressing and hardening is complete the gear blank will present the appearance in cross section shown in Figure 3. The rings 14 and 18 form the rim 55 section and the central portion of the discs 16 form the web section.

The blank is now ready to be machined and the machining may be accomplished in the usual way. For example, the gear teeth 60 18 may be generated by the hobbing process. Ordinarily it will also be necessary to cut out a central aperture 20 for accommodating the shaft on which the gear is to be mounted.

65 It will be observed that as a result of my method there is no waste of material; also

that all the layers lie in parallel planes. There is no distortion or warping either of the rings 14, 18 or of the discs 16. The result is that there is nothing to create any tendency for the gear section to lack uniformity. On the contrary not only will a given diametral section be symmetrical, but all diametral sections will be alike. The mold instead of having a tendency to throw the planes out of true will have a tendency 70 to keep them true. The result is that the gear will be perfectly balanced about its central axis and will always run true. This will prevent it from being noisy and will increase its life. 75

80 In Figure 6, I have illustrated diagrammatically the appearance of the component parts of the finished gear, the layers of woven fabric being impregnated with the binder. The appearance of the parts in this figure is 85 exaggerated in order to render the construction more apparent.

Having thus described my invention what I claim as new and desire to secure by Letters Patent is:—

89 1. The process of making gears having webs of reduced thickness, consisting in assembling flatwise a plurality of circular layers of woven fabric of the full diameter of the gear in all directions, and a plurality of flat rings of woven fabric upon both sides of the first mentioned layers, said rings being superposed and forming the rim portion of the gear, said rings and layers being impregnated with a binder capable of hardening under heat, heating said rings and layers, and simultaneously compressing said rings and layers in a direction normal to their surfaces, and to such extent as to produce a greater aggregate reduction of thickness in the rim than in the web portion. 105

110 2. The process of making composite gears having a web of reduced thickness, the process consisting in assembling in parallel planes a plurality of layers of woven fabric, the outer layers consisting of rings co-extensive with the rim section and the inner layers extending also inward toward the center to form the web section, saturating the 115 layers in a binder capable of hardening under heat, and compressing the rim portion and the web portion separately to prevent distortion of the fabrics from their true plane.

120 3. The process of making composite gears having a web of reduced thickness, the process consisting in assembling in parallel planes a plurality of layers of woven fabric, the outer layers consisting of rings co-extensive with the rim section and the inner layers extending also inward toward the center to form the web section, saturating the 125 layers in a binder capable of hardening under heat, and compressing the rim portion and the web portion separately but si- 130

multaneously, and finally bringing the two pressures to approximately the same degree of intensity per unit area, the pressures being exerted in a direction perpendicular to the plane of the gear.

4. The process of making gears having webs of reduced thickness, consisting in assembling a plurality of circular discs of woven fabric in parallel planes, superposing 10 on both sides of said discs rings of woven fabric arranged in parallel planes and having outer diameters of substantially the same outer diameter as the discs, impregnating the rings and layers with a phenolic binder 15 capable of hardening under heat, heating said rings and layers, exerting pressure thereon normal to their surfaces, and confining said rings and layers circumferentially, the heating and pressing occurring simul- 20 taneously, and the rim portion of the gear

blank receiving a greater total compression than the web portion.

5. The process of making gears having webs of reduced thickness, consisting in assembling a plurality of circular discs of woven fabric in parallel planes, superposing on both sides of said discs rings of woven fabric arranged in parallel planes and having outer diameters of substantially the same outer diameter as the discs, impregnating the rings and layers with a phenolic binder capable of hardening under heat, heating said rings and layers, exerting pressure thereon normal to their surfaces, and confining said rings and layers circumferentially and the rings at their internal diameters. 30 35

In witness whereof, I have hereunto subscribed my name.

LOUIS T. FREDERICK.